

Patented June 12, 1923.

1,458,592

# UNITED STATES PATENT OFFICE.

CARL P. OLSON, OF IRVINGTON, NEW JERSEY.

## WRAPPING TISSUE.

No Drawing.

Application filed April 17, 1922. Serial No. 554,181.

To all whom it may concern:

Be it known that I, CARL P. OLSON, a citizen of the United States, residing in the town of Irvington, county of Essex, and 5 State of New Jersey, have invented certain new and useful Improvements in Wrapping Tissues, of which the following is a specification.

My invention relates to wrapping tissues, 10 and particularly to film-like wrappers of cellulose acetate tissue.

It has for its objects the provision of a thin, flexible, strong tissue which shall be non-porous, non-hygroscopic, non-inflammable, transparent and cheap, and adapted 15 for all uses as a wrapping sheet for which tissues of paper or gelatine are now employed, but that shall be stronger than such tissues of equal thickness; that shall be of 20 transparency equal to that of gelatine tissues of equal thickness, but, unlike such gelatine tissues, shall be non-brittle and highly flexible; that shall not be absorptive of moisture and liable to consequent deterioration, 25 as is a gelatine tissue; that shall be impervious to dust and dirt; that shall afford a measure of protection against fire from flame, and that shall be capable of affording 30 sanitary protection by its amorphous and non-porous texture to a contained article.

To these ends my invention consists in a wrapper of flame-retarding tissue made from an organic ester or esters of cellulose, such as esters of cellulose with the paraffin series 35 of acids, such as acetic acid; or from cellulose or cellulosic compounds or derivatives with alcohol radicals, such as the ethyl or other alkyl celluloses, benzylcellulose or other arylcellulose esters, for the purposes 40 specified, as a new article of manufacture.

While nitrocellulose and nitrocellulose compounds, and those bodies going under the general name of viscose have been proposed for similar purposes, I disclaim their use 45 in this connection as also the relatively inflammable esters of cellulose and mixtures or combinations in which they are an essential constituent or compound; together with any cellulose, cellulose derivative or cellulosic 50 compounds or ester prepared therefrom which contain any acid radical adapted to render such compound inflammable.

In the preferred form of my invention I employ, as raw materials, cellulose, as cotton or tissue paper; glacial acetic acid, glacial; acetic anhydride, and a catalyst such as

a very small amount of sulfuric acid or zinc chloride. The method of manufacture and quantities of each may be as follows: Take

|                                 | Parts by weight. |
|---------------------------------|------------------|
| Cellulose                       | 100              |
| Glacial acetic acid             | 350              |
| Acetic anhydride (80% strength) | 250              |
| Sulfuric acid                   | 2                |

Total 702

The foregoing components, excepting the cellulose, are placed in a mixer, and agitated. 70 During agitation the cellulose, properly dried, is fed in small quantities to the mix. After the cellulose has all become incorporated, which requires from 2 to 3 hours, the temperature being meanwhile maintained 75 below 20° C., the cellulosic compound, will be found, upon test in chloroform free from ethyl alcohol, to be substantially insoluble. The process is then continued until the product, after precipitation and washing until 80 neutral, is found to dissolve in warm, pure chloroform but not to dissolve in pure acetone.

The product is then partially hydrated by the addition of about 3% of water, added in 85 small amounts at a time. The hydrated product, a heavy, viscous, clear liquid, is then maintained at a temperature of 25° to 30° C. for several days, and until a sample is found to have lost its solubility in warm 90 chloroform and to have acquired a complete solubility in cold or warm pure acetone. When this stage of ripening is reached, the batch is precipitated by added water, the batch being stirred during such addition of 95 water thereto, and such washing is continued to neutrality in a manner similar to the treatment of pyroxylin in beaters, except that the cellulose acetate is already in a state of fine subdivision from precipitation. This pre-

cipitated and washed cellulose acetate is next hydro-extracted, and flowed, or otherwise spread, as by the methods and apparatus of my U. S. Letters Patent No. 1,387,068, granted me August 9, 1920, upon a 100 film-forming medium, and dried at a moderate temperature in the form of a thin tissue of desired dimensions. While I am aware that it has been proposed to form a box and lid therefor of acetyl-cellulose and 105 to line tubes or containers to make them fluid-tight with a film of cellulose acetate, or

to coat a paper receptacle with a cellulose ester solution to make same resistant to moist alkalis, I believe it is broadly novel to produce a flat self-supporting sheet of acetyl cellulose, having the superficial dimensions in which paper is made, for example, double elephant writing or double royal printing, and of the thinness and fineness of the finest grade of tissue paper, which sheet is adapted 5 by its size and quality to the utilities for which the finer grades of wrapping paper are customarily used.

10 The tissue produced is free from odour, non-porous, pliant, transparent, and slow-burning, and otherwise embodies the desired qualities and characteristics heretofore set forth as the desired objects to be attained 15 and realizes all the beneficial features of par-

ticular utility and advantage specified. In the subjoined claim, by the phrase "wrapping sheet of tissue paper character," or the like, I desire to be understood as intending a flat sheet of self-supporting strength, of the thinness and fineness of tissue paper and of dimensions approximately those standard sizes in which tissue paper is customarily manufactured.

Having thus described my invention and the method practiced and means employed by me in producing the same in the form believed by me to be its best embodiment, I claim:

As a new article of manufacture, a wrapping sheet of tissue paper character composed of acetyl cellulose.

CARL P. OLSON.